

## UNITED STATES PATENT OFFICE.

F WALTER GUIBERT, OF DETROIT, MICHIGAN.

## METHOD OF ANNEALING OR HEAT-TREATING STEEL OR OTHER METALS.

No Drawing.

Application filed October 24, 1925. Serial No. 64,692.

My invention relates to a method of annealing or heat-treating steel or other metals. It has to do particularly with a novel method of annealing steel or other metals in such a manner that the steel will be properly normalized and annealed without subjecting the surface thereof to oxidation and discoloration during the treating process. There is also a heavy oxide formed on metals, especially alloy metals when the same are heat treated by raising to high heat, then hardened by quenching. Then, as a rule, they are drawn back, or normalized or tempered at a lower heat. This produces a still heavier oxide. It is the object of my invention to avoid the formation of the oxide by performing these operations in a vacuum or a rarified atmosphere.

In the past, especially in the art of annealing steel and other similar metals, many different methods have been resorted to in an attempt to improve the physical properties of the steel and remove the strains and other objectionable characteristics which are always set up during the initial rolling or formation of the article to be annealed. Some of these methods have contemplated the placing of the article to be treated in a uniform compartment containing a neutral atmosphere. Other methods have involved the placing of the steel or other metals in a compartment or annealing box and surrounding the steel with iron filings, carbon monoxide, or other non-oxidizing gases.

Many other methods have been utilized in the heat-treating of steel and some of these methods have been commercially successful in the proper treating of the core of the article. However, none of these methods have been completely successful in that they have invariably failed to prevent the formation of scale and discoloration of the surface of the article during the annealing or heat treating process.

I have discovered, that by subjecting the steel article, or other metals to be treated, to a vacuum and then heating the metal to the proper degree as required, while the metal is subjected to the vacuum, oxidation and discoloration of the surface may be effectively prevented. My novel method may be accomplished in various ways and by various apparatus, all of which are well

known in the art, and do not require drawings for illustration. For instance, the heating compartment may be filled with the metals to be heat-treated, the air exhausted by a vacuum pump, or the compartment may be filled with steam which may be condensed, or drained out, or other suitable means for securing a vacuum may be employed. The compartment is sealed, and the sealed compartment placed in a suitable furnace for heating the metals. The metal in the vacuum compartment may be heated by conduction as directly by electric resistance.

Where it is desired to anneal and heat-treat cold rolled strip or sheet steel or copper and brass by a continuous action, the entire reel of metal together with the receiving reel may be placed in a compartment which may be subjected to vacuum and the metal in passing from one reel to the other reel is subjected to heat by conduction as by electric resistance.

Many other forms of construction may be utilized in practising my method. However, the present invention is not directed to the apparatus or details for effecting the vacuum or for heating the steel, but broadly to the method of subjecting the metal to be treated to a vacuum during the treating process.

It will be understood that the degree of vacuum in the annealing or vacuum chamber need not be fixed to effect the successful working of my method. The oxidation and discoloration will be prevented to a marked degree by even a small amount of vacuum, but it will also be understood that by producing a large degree of vacuum in the heat-treating chamber, and by maintaining this vacuum during the heating process, and cooling off, that practically all tendency of the surface of the steel or other metal to oxidize or discolor will be prevented. In other words, the improvement in the physical properties of the metal and the neutralization of the oxidizing influence to effect the color and texture of its surface will depend proportionately on the degree of vacuum obtaining in the annealing chamber or around the metal during the annealing process or heat treating process.

It will be understood that in using the term "vacuum" in the claims I do not limit

myself to a theoretically perfect vacuum, but other metals adapted to be hardened by heat-treating, which consists in heating the metal to the proper degree and then quenching to effect the heat-treating thereof, and surrounding the metal with a vacuum to prevent oxidization and discoloration of the surface during the entire heat-treating process.

What I claim is:

- 5 1. The method of heat-treating steel or other metals adapted to be hardened by heat-treating which consists in heating the metal to the proper degree and then quenching, the metal being maintained in a vacuum during the entire process.
- 10 2. The method of heat-treating steel or

In testimony whereof I have affixed my signature.

F WALTER GUIBERT.